

# United States Patent Office

2,838,396

Patented June 10, 1958

1

2,838,396

## METAL PRODUCTION

Thor N. Rhodin, Jr., Wilmington, Del., assignor to E. I. du Pont de Nemours and Company, Wilmington, Del., a corporation of Delaware

No Drawing. Application November 14, 1956  
Serial No. 622,019

10 Claims. (Cl. 75—174)

This invention relates to novel niobium-base alloys and more particularly to improved niobium-aluminum-chromium alloys exhibiting unusual strength and oxidation resistance under extreme high temperature service conditions.

For an alloy to be useful as a material of construction in applications such as jet and diesel engines, atomic power reactors, gas turbines, turbine blades or buckets and nozzle guide vanes for turbines, dies for high temperature metal working, high temperature reactors, and the like, it must possess satisfactory high melting point, strength and oxidation resistance properties and also must be amenable to fabrication. Disadvantageously, prior metals and alloys lack these essential qualities to render existent a real need for an alloy capable of satisfactory performance under the service conditions encountered in applications of the type mentioned.

It is among the objects of this invention to overcome these disadvantages of prior metallic construction materials and to provide a novel alloy composition particularly adapted and useful in attaining these objects. Further objects of the invention include the provision of an improved, workable alloy composition having superior strength and oxidation-resistance characteristics at relatively high, above 1000° C., temperatures; the provision of niobium-base alloy useful in the applications mentioned and adapted to withstand high mechanical stresses at temperatures above 1000° C.; to provide a niobium-aluminum-chromium alloy which is desirably resistant to oxidation at temperatures considerably above 800° C., and ranging from 1000–1300° C. and higher, and which is satisfactorily ductile and readily amenable to mechanical fabrication under hot or cold working or drawing conditions, including hot swaging, hot rolling, forging, hot pressing extrusion, etc.; to provide a niobium-aluminum-chromium alloy having requisite, superior hardness properties and which does not require thermal treatment to develop maximum strength at elevated temperatures; to provide an alloy composition of the type mentioned having superior fatigue, tensile and rupture properties at relatively high temperatures and which undergoes no significant permanent dimensional changes upon subjection to prolonged exposure under extreme temperature conditions; and to provide a niobium-aluminum-chromium alloy composition having unique, especially protective surface layers of reaction products and which advantageously exhibits such chemical and mechanical attributes as desired adherence, nonpermeability, dimensional stability, nonvolatility and minimum film thickness when exposed to corrosive atmospheres at high temperatures. Other objects and advantages of the invention will be evident from the ensuing detailed description.

These and other objects are realized by the alloys of this invention which contain as essential ingredients at least 55% by weight of niobium, about 1–20% by weight of aluminum and about 1–30% by weight of chromium. In combination with the elements mentioned, there may be added from 0–35% by weight of one or more of the elements cobalt, nickel, tungsten and zirconium, from 0–5% by weight of one or more of the elements beryllium, manganese, silicon, thorium and vanadium, and from 0–2% by weight of one or more of the elements boron, carbon, calcium and cerium to impart to the alloy certain desired characteristics, such as the properties of protective oxide scale or the special metallurgical response of the alloy to working, such as for example, heat treatment or fabrication. When mixtures of two or more of such added elements are employed, the total quantity used from said 0–5% range should not exceed 15% by weight; and from said 0–2% range, should not exceed 5% by weight.

In a more specific and preferred embodiment, my novel alloy composition contains from about 55% to 80% by weight of niobium, from 4% to 25% by weight of aluminum, and from 8% to 30% by weight of chromium, with the amounts of added elements present being in the following ranges and total amounts: 0–20% by weight of one or more of the elements cobalt, nickel, tungsten and zirconium, the total of this group not to exceed 35%; 0–5% by weight of one or more of the elements beryllium, manganese, silicon, thorium and vanadium, the total of this group not to exceed 15%; and from 0–2% by weight of said boron, carbon, calcium and cerium elements, the total of this group not to exceed 5%.

My improved alloys can be prepared in accordance with conventional procedures and through recourse to known melting and casting techniques. Thus, the individual metals can be melt-cast together and the melt allowed to cool and solidify into a desired shape. The melting operation can be carried out in an arc melting furnace provided with consumable or non-consumable electrodes, or by subjecting the charge to induction heating in a skull or crucible type of container. One useful form of arc melting furnace comprises that having an integral, water-cooled copper crucible in which the charge can be melted and solidified, such as that described by W. Kroll in "Transactions of the Electrochemical Society," vol. 78, pages 35–47, 1940. Alternatively, a compressed, consumable arc electrode type melting furnace can be employed, such as described in U. S. 2,640,860 to S. A. Herres, as can the combination of a nonconsumable and consumable electrode type of double melting furnace described in U. S. 2,541,764, to S. A. Herres. A continuous feed type of furnace can also be used, such as described in U. S. P. B. Report 111,083. Whatever type furnacing means is employed, care should be exercised in the melting and casting operation to protect the molten metal from normal atmospheric contamination through contact with oxygen, nitrogen, etc. This can be prevented by conducting the operation under a vacuum or an atmosphere of an inert gas, such as argon, helium, etc.

The individual metals charged to the melting furnace can be in any desired form, e. g., powder, granular, shot, wire or sponge, and should be of commercially acceptable purity to insure production of a satisfactorily pure alloy product. The cast material obtained will consist of a workable metal having excellent strength and oxidation resistance at high temperatures, and will be eminently suitable for use as a material of construction in high temperature equipment designed to operate at temperatures beyond the limits of present equipment constructed of the best high temperature alloys.

Advantageously, my alloys will exhibit high strength at temperatures ranging from 1000–1300° C. or higher, at which temperatures other high temperature alloys lose strength, become plastic or melt, will be characterized by especially protective layers of reaction products on or below the metal surface consisting of compounds of the alloy with oxygen, nitrogen, hydrogen, carbon, sulfur or halogens or compounds thereof present in the atmos-

sphere; and will be found to have been adjusted to produce especially protective surface layers containing combinations of the compounds mentioned with themselves, such as spinel oxides or with each other, such as mixed oxides-nitrides to provide very high resistance to deleterious attack of the alloy by the surrounding gases. The data given below demonstrate the properties of the alloys in respect to high temperature oxidation resistance. Their performance with reference to a balance between oxidation resistance and fabricability is determined by the relative proportions of the alloying elements. Since these two properties tend to oppose each other, the ranges in composition given were chosen on the basis of establishing an optimum compromise between them.

To a clearer understanding of the invention, the following specific examples are given. These are only illustrative and are not to be considered as limiting the scope and underlying principles of the invention. As will be noted many of the aluminum-chromium-modified niobium-base alloys given are characterized by unusually high niobium content, and in the preferred 55-80% range. In addition, the protective films characteristic of oxidation at 1000° C. and 1300° C. often contain relatively little niobium oxide but are often substantially enriched in aluminum oxide. This inversion in the niobium-aluminum ratio between the alloy and the protective films is especially unique for these alloys and comprises a novel and outstanding feature of my invention.

#### EXAMPLE I

A granular mixture of 65% by weight niobium, 5% by weight aluminum, and 30% by weight of chromium was charged into a water-cooled, copper crucible of an arc melting furnace of the type described above and the metals heated under an atmosphere of helium to effect complete fusion of the metal charge. When the charge became liquefied the furnace was turned off and the melt was allowed to cool in the inert atmosphere, discharged from the crucible and was tested for resistance to high temperature oxidation in the following manner:

A coupon was cut from the "as cast" button and heated at 1000° C. and 1200° C. for 24 hours in a helium atmosphere. The sample was then heated to 1000° C. and 1200° C. in a recording thermobalance in flowing air for 24 hours. Oxidation rates were followed by making continuous measurements of weight change while the sample was at a controlled temperature without interruption of the test during the 24-hour period. Non-volatility of surface compounds under these test conditions was also determined by measuring no weight change when exposed to pure helium.

Upon termination of the oxidation test, the sample was cooled and the protective character of the surface layers determined by metallographic examination and chemical analysis. In addition, the effect of oxidation on the metal alloy itself was examined by the same methods. It had an oxidation rate of 0.15 mg./sq. cm./hr. after 24 hours at 1000° C. and a rate of 0.26 mg./sq. cm./hr. after 24 hours at 1200° C. A specimen of pure niobium metal, subjected to the same test had, in contrast, an oxidation rate of 22.0 mg./sq. cm./hr. after 24 hours at 1000° C., and 68 mg./sq. cm./hr. at 1200° C.; and, in some cases, was completely converted to the oxide after treatment at 1000° C. and 1200° C. The specimen of this example, on the other hand, was covered with a very thin, especially adherent protective oxide layer which corresponded to less than 0.04% conversion of the metal at 1000° C. and less than 0.10% conversion at 1200° C. This layer showed outstanding resistance to spalling when the specimen was heated to 1000° C. and 1200° C. and then cooled to room temperature.

#### EXAMPLE II

An alloy was prepared in the same manner as in Example I except that its composition was 67% by weight

niobium, 5% by weight aluminum, 26% by weight chromium and 2% by weight nickel.

After testing as described in Example I, its oxidation rate was 0.05 mg./sq. cm./hr. after 24 hours at 1000° C. and 0.16 mg./sq. cm./hr. after 24 hours at 1200° C. This corresponded to less than 0.03% and 0.08% conversion of the metal at 1000° C. and at 1200° C., respectively. The adherence and coherency of the oxide film in this alloy was found to be exceptional, particularly upon heating and cooling from 1200° C. or from 1000° C. to room temperature.

#### EXAMPLE III

An alloy was prepared as described in Example I except that its composition was 75% by weight niobium, 15% by weight aluminum, 10% by weight chromium. A coupon was cut from the cast material and upon heating and testing as in Example I had the properties shown in Table I below. Upon forging and machining the remaining casting into a nozzle element and employing such nozzle for spraying  $MgCl_2$  at a temperature above 800° C. in a chemical process, the alloy exhibited excellent high temperature oxidation resistance characteristics to prove highly useful in such application.

#### EXAMPLE IV

An alloy was prepared as in Example I except that its composition was 65% by weight niobium, 20% by weight aluminum, 15% by weight chromium. Upon subjecting 30 a coupon cut from the as cast material to the test described in Example I, it had characteristics as shown in Table I below.

#### EXAMPLE V

An alloy was prepared as described in Example I except that its composition comprised 56% by weight niobium, 10% by weight aluminum, 19% by weight chromium and 15% by weight cobalt. Upon testing as in Example I, it had the properties shown in Table I below.

#### EXAMPLE VI

An alloy was prepared as described in Example I except that its composition comprised 76% by weight niobium, 10% by weight aluminum, 10% by weight chromium and 4% by weight tungsten. Its characteristics 45 are shown in Table I below.

#### EXAMPLE VII

An alloy was prepared as described in Example I except that its composition comprised 63% by weight niobium, 15% by weight aluminum, 20% by weight chromium, and 2% by weight cerium. Its characteristics 50 are shown in Table I below.

#### EXAMPLE VIII

An alloy was prepared as described in Example I except that its composition comprised 59% by weight niobium, 10% by weight aluminum, 10% by weight chromium, 15% by weight nickel, 4% by weight tungsten and 2% by weight cerium. Its characteristics are shown 60 in Table I below.

Table I

| Example                                          | Oxidation Rate (mg./sq. cm./hr.) |           | Adherence of Oxide Scale |
|--------------------------------------------------|----------------------------------|-----------|--------------------------|
|                                                  | 1,000° C.                        | 1,200° C. |                          |
| Control 100% Nb                                  | 22                               | 68        | Very Poor.               |
| I-65% Nb, 5% Al, 30% Cr                          | 0.15                             | 0.26      | Good.                    |
| II-67% Nb, 5% Al, 26% Cr, 2% Ni                  | 0.05                             | 0.16      | Excellent.               |
| III-75% Nb, 15% Al, 10% Cr                       | 0.05                             | —         | Do.                      |
| IV-65% Nb, 20% Al, 15% Cr                        | 0.03                             | —         | Do.                      |
| V-56% Nb, 10% Al, 19% Cr, 15% Co                 | 0.01                             | 0.06      | Do.                      |
| VI-76% Nb, 10% Al, 10% Cr, 4% W                  | 0.05                             | 0.17      | Do.                      |
| VII-63% Nb, 15% Al, 20% Cr, 2% Ce                | 0.05                             | 0.14      | Good.                    |
| VIII-59% Nb, 10% Al, 10% Cr, 15% Ni, 2% Ce, 4% W | 0.02                             | 0.05      | Excellent.               |

As noted, the alloys of this invention are useful as materials of construction in all applications requiring strength and a corrosion-resistant metal. Hence, while particularly useful in high temperature equipment which must operate above 800° C., such as jet engine parts, nuclear reactors, gas turbine parts, etc., my novel alloys due to their outstanding properties, including nonbrittleness and adaptability for successful fabrication by hot swaging or rolling, forging, hot pressing or extrusion, are not restricted to such applications nor to any particular equipment described or referred to herein.

When recourse is had to the use of cobalt, nickel and zirconium in combination with niobium, aluminum and chromium, from about 1-30% by weight of such elements can be employed; when beryllium, manganese, silicon, thorium, vanadium and tungsten are used an amount from 0.1-5% by weight can be employed; while from 0.1-2% by weight of boron, carbon and cerium can be used.

Although I prefer to employ metals exhibiting relatively high purity, some variance in purity properties can be tolerated. Thus, the alloys of the examples and those tested were obtained from commercially available niobium, aluminum and chromium containing less than 1% incidental impurities. Commercial niobium usually contains tantalum (in amounts up to 5%) which is difficult to detect and separate. Therefore, the niobium contemplated for use herein may contain small amounts (0.1 to 5.0%) of tantalum as well as iron, oxygen and possibly silicon as impurities. Elimination of certain of these impurities (silicon, oxygen) or enhancement of others (tantalum, iron) may improve oxidation resistance significantly.

Since many changes and modifications can be made in the invention without departing from its underlying principles, it will be understood that it is not restricted to the above detailed description, but only as defined in the appended claims.

I claim:

1. A niobium-base alloy containing as essential ingredients at least 55% by weight of niobium, from 1-20% by weight of aluminum and from 1-30% by weight of chromium.

2. An oxidation-resistant niobium-base alloy composition containing from about 55-80% by weight of niobium, from about 4-20% by weight of aluminum, and from about 8-30% by weight of chromium, said alloy being adapted to withstand prolonged exposure at a temperature above 800° C.

3. A niobium-base alloy containing at least 55% by weight of niobium, from 1-20% by weight of aluminum, from 1-30% by weight of chromium, and in combination therewith from 0-35% by weight of an element selected from the group consisting of cobalt, nickel, tungsten,

zirconium, from 0-5% by weight of an element selected from the group consisting of beryllium, manganese, silicon, thorium and vanadium, and from 0-2% by weight of an element selected from the group consisting of boron, carbon, calcium and cerium.

4. An oxidation-resistant niobium-base alloy composition containing from about 55-80% by weight of niobium, from about 4-20% by weight of aluminum, from about 8-30% by weight of chromium, and from 1-20% by weight of nickel, said alloy being adapted to withstand prolonged exposure at a temperature above 800° C.

5. An oxidation-resistant niobium-base alloy composition containing from about 55-80% by weight of niobium, from about 4-20% by weight of aluminum, from about 8-30% by weight of chromium, and from 1-20% by weight of cobalt, said alloy being adapted to withstand prolonged exposure at a temperature above 800° C.

6. An oxidation-resistant niobium-base alloy composition containing from about 55-80% by weight of niobium, from about 4-20% by weight of aluminum, from about 8-30% by weight of chromium, from 1-20% by weight of nickel, from 0.1-5% by weight of tungsten, and from 0.1-2% by weight of cerium, said alloy being adapted to withstand prolonged exposure at a temperature above 800° C.

7. An oxidation-resistant alloy containing, by weight, about 67% niobium, 5% aluminum, 26% chromium and 2% nickel.

8. An oxidation-resistant alloy containing, by weight, about 56% niobium, 10% aluminum, 19% chromium, 15% cobalt.

9. An oxidation-resistant alloy containing, by weight, about 59% niobium, 10% aluminum, 10% chromium, 15% nickel, 4% tungsten and 2% cerium.

10. A niobium-base alloy containing at least 55% by weight of niobium, from 1-20% by weight of aluminum, from 1-30% by weight of chromium, and in combination therewith from 0-35% by weight of at least one element selected from the group consisting of cobalt, nickel, tungsten, zirconium, the total of the elements of this group not to exceed 35%; from 0-5% by weight of at least one element selected from the group consisting of beryllium, manganese, silicon, thorium and vanadium, the total of the elements selected from this group not to exceed 15%; and from 0-2% by weight of at least one element selected from the group consisting of boron, carbon, calcium and cerium, the total of the elements selected from this group not to exceed 5%.

#### References Cited in the file of this patent

"Initial Investigation of Niobium and Niobium-Base Alloys," Saller, Stacy, Porembka, AEC, BMI-1003, May 23, 1955.